

May 5, 1936.

J. L. DOSTAL

2,039,397

METHOD OF FORMING TAPPETS

Original Filed Sept. 28, 1929 2 Sheets-Sheet 1



INVENTOR

Joseph L. Dostal

BY

Hansen, Hickey, Pierce & Hann.  
ATTORNEYS.

May 5, 1936.

J. L. DOSTAL

2,039,397

METHOD OF FORMING TAPPETS

Original Filed Sept. 28, 1929 2 Sheets-Sheet 2



INVENTOR  
Joseph L. Dostal.

BY  
Harness, Wickes, Pierce & Hamm  
ATTORNEYS.

Patented May 5, 1936

2,039,397

# UNITED STATES PATENT OFFICE

2,039,397

## METHOD OF FORMING TAPPETS

Joseph L. Dostal, Flint, Mich., assignor to Eaton-Erb Foundry Company, a corporation of Michigan

Original application September 28, 1929, Serial No. 395,949. Divided and this application July 17, 1933, Serial No. 680,774

6 Claims. (Cl. 22—213)

This invention relates to a method of forming tappets and particularly to an improved method of forming cast iron tappets for use in connection with internal combustion engines, the principal object being the provision of a new and novel method by means of which an improved tappet may be produced economically in quantities, and is a division of my application for Letters Patent of the United States for improvements in Means for producing hardened cast iron valve tappets, filed September 28, 1929, and serially numbered 395,949.

Objects of the invention include the provision of a method of forming cast iron valve tappets including casting the face of the tappet against a chill and controlling the temperature of the mold and/or chill so as to obtain the desired hardness of the tappet face and/or softness of the tappet body; a method of casting a cast iron tappet in a metallic mold in such a manner as to obtain a chilled face for the tappet and a relatively soft body therefor; a method of producing quantities of cast tappets by the use of a metallic mold having a movable chill plate by the use of which the temperature of the chill plate may be controlled so as not to exceed a predetermined maximum necessary to obtain the desired hardness of the chilled face of the tappet; a method of producing a plurality of cast iron tappets by the use of a metallic mold having a removable chill plate forming that face of the mold adapted to produce the face of the tappet, and replacing the chill plate by a cooler chill plate when the temperature of the chill plate being employed in the casting operation approaches a predetermined high temperature; and the continuous production of cast iron valve tappets by the employment of a cast iron of predetermined composition in a metallic mold, having certain walls of the mold depressions insulated against the transfer of heat thereto, and certain other walls of the depressions formed by a chill plate so constructed as to permit control of the temperature thereof.

The above being among the objects of the present invention, the same consists of certain novel steps of operation in the manufacture of cast iron valve tappets to be hereinafter described with reference to the accompanying drawings, and then claimed, having the above and other objects in view.

In the accompanying drawings which illustrate apparatus suitable for the satisfactory carrying out of the present invention, and in which like numerals refer to like parts throughout the several different views,

Figure 1 is a side elevational view of a conventional form of valve tappet which may be cast according to the present invention, showing a part of the gate formed in the casting operation attached thereto.

Fig. 2 is a vertical sectional view taken centrally through a mold suitable for use in connection with the present invention, as on the line 2—2 of Fig. 3, and giving an elevational view of the inner face of one of the mold halves, together with the chill plate employed in connection therewith.

Fig. 3 is a vertical sectional view taken transversely to the length of the mold shown in Fig. 2 as on the line 3—3 of Fig. 2, and illustrating one of the mold cavities as being filled with metal.

Fig. 4 is a plan view of the mold shown in Figs. 2 and 3, without the chill plate, and with the mold halves slightly separated.

Fig. 5 is a fragmentary perspective view of one end of the chill plate used in connection with the mold indicated in Figs. 2 to 4, inclusive.

It is, of course, well understood in the art that valve tappets for internal combustion engines formed from white cast iron and including a chilled face and relatively soft body are desirable both from the standpoint of economy in production and efficiency and long life in use.

The prior practice in the production of such valve tappets has been to provide a sand mold having a chill plate inserted for forming the face of the tappet, and in such method of production it is possible to obtain a satisfactory uniformity of product in quantity production. In such case, however, due to the fact that the sand cores or molds are destroyed after each casting operation, the production cost of the tappets is higher than desired, and one of the main objects of the present invention is to eliminate the heretofore relatively high expense in connection with the use of sand cores or molds. This saving, in accordance with the present invention, is primarily accomplished by the use of permanent metallic molds which may be used over and over again and which thus result in a very slight charge per tappet for molding costs.

In employing a permanent metallic mold for this purpose, however, it will be apparent that the molds themselves tend to absorb a very material amount of heat from the metal being cast, and while this is of advantage in certain respects, it is also a decided disadvantage in other respects. The advantages are that the body of the mold in absorbing heat from the molten metal being cast tends to reduce the transfer of heat

- between the metal and the mold, and thereby aids in obtaining a relatively soft body for the tappet which is of advantage, but even in such cases it has been found that it is necessary to provide some form of heat insulation between the body of the tappet and the body of the mold to further reduce the heat transfer and to insure the proper softness of the metal in the body of the tappet.
- 10 The disadvantage of the absorption of heat by the mold from the metal being cast is that in order to provide the desired chilling of the face of the tappet, the surface of the mold forming the face of the tappet must be maintained at a relatively low temperature or otherwise the desired degree of hardness of the face of the tappet will not be obtained. Accordingly, the adaptation of permanent molds to the art of casting valve tappets having chilled faces creates several difficulties which are overcome in accordance with the present invention. Briefly stated, in accordance with the present invention the metal which is to form the body portion of the tappet is insulated against excessive transfer of heat to the body of the mold by providing the corresponding surfaces of the mold depression with a relatively thin coating of heat insulating material capable of satisfactorily withstanding the high temperatures of the metal being poured, and providing a separate member adapted to form the face of the tappet and so cooling this member as to limit its maximum temperature or, if necessary, removing such member after its temperature has attained a predetermined high value and replacing it with another like and cooler member. The above method, particularly where the temperature of the mold itself is controlled, results in a product of uniform quality in quantity production.
- 40 Referring now to the accompanying drawings, as a matter of illustration only, in Fig. 1 is shown one conventional form of tappet which may be formed in accordance with the present invention. This tappet, generally known as the "mushroom" type, comprises a cylindrical body portion 10 having an enlarged head 12 connected thereto through an undercut portion 14, and a reduced end 16 opposite the head 12 provided with flats 18 on diametrically opposite sides thereof for the purpose of allowing ready engagement with a wrench or other tool. In casting these tappets they are gated at the end 16 and in Fig. 1 a gate 20 is shown attached thereto as in the manner in which the tappet is removed from the mold.
- 45 Referring to the drawings, it will be noted that the mold shown comprises two main halves 22 and 24 having matching planar faces and, for ease in manufacture, each half is made up of a plurality of superposed sections each including a bottom section 26, a top section 28 and an intermediate section 29. These sections of each half are maintained in alignment by dowel pins 30 and secured together as a unit by screws 31. Dowel pins 32 secured to the half 24 and fitting 50 within openings 33 in the half 22 serve to maintain alignment of the halves 22 and 24 during operation. Cooperating cavities 34 are formed in the opposed faces of the intermediate members 29 of the halves 22 and 24 simulating the shape of the desired tappet, but preferably of slightly larger diameter than the desired tappet due to the preferred use of a heat insulating coating to be more fully disclosed. The depressions 34 open upon the lower face of the sections 29 at 55 which point the head 12 of the tappet is adapted to be formed. Matching depressions 35 forming gates for the cavities 34 are formed in the opposed faces of the sections 28. A channel 36 is formed at the top of the sections 28 between the opposed faces thereof and is connected by means of a triangularly shaped trough 38 with the gate depressions 35, the trough 38 thus serving as a sprue. It will be noted from an inspection of Fig. 2 that the trough 38 tapers from a minimum depth at one end of mold to a maximum depth 10 at the opposite end thereof so that when metal is poured into one end of the trough 36 it will successively fill successive gates 35 and corresponding cavities 34. It is to be understood, of course, that the channel 36 and trough 38 stop short of opposite ends of the mold halves 22 and 24.
- 15 A channel 40 is formed between the upper ends of the opposed faces of the sections 26 and extends completely through the mold halves 22 and 24 from end to end. Relatively loosely received in the channel 40 is a chill member, plate or block 42 which substantially completely fills the channel 40 and the upper surface of which substantially abuts the lower faces of the sections 29 thereby to serve as a closure for the bottom of the depressions or cavities 34 and acts to serve as face of the cavities 34 defining the face of the head 12 of the tappet although, due to the necessary looseness of fit of the chill plate 42 in 25 the channel 40 a slight amount of clearance may be present between the top of the chill plate 42 and the sections 29 which may act to permit the escape of gas from the mold cavities. Dowels 44 are threaded into the half 22 and project through 30 suitable openings 46 in the half 24. These dowels project through the lower portion of the channel 40 and the chill plate 42 is provided with transverse grooves 48 in its lower surface of reception of the dowel pins 44 which thereby maintains the 40 chill plate 42 against inadvertent longitudinal shifting movement and serve as guides therefor when the mold halves are separated.
- 20 The walls of the depressions 34, gates 35, channel 36 and trough 38 are preferably provided with 45 a relatively thin adherent coating 50 of heat insulating refractory material of the type disclosed in United States Patents No. 1,453,593; 1,492,694; 1,506,130; 1,560,838 or 1,568,234. None of this coating however is applied to the chill plate 42 50 for it is this plate which is adapted to form the chilled face for the tappet and consequently which is designed to chill the metal cast against it as rapidly as possible. Before each pouring operation, however, all of these surfaces including the 55 surface of the chill plate 42 are preferably provided with a coating of lampblack in the manner referred to in United States Patent No. 1,492,694.
- 25 A thermo-couple 52 embedded in an end of the chill plate 42 and extending to a point directly 60 below one of the depressions 34 is connected by leads 54 to a device 56 adapted to indicate the temperature at the point of the thermo-couple.
- 30 In operation, the mold halves 22 and 24 are mounted in a suitable molding machine (not 65 shown) so that the cavities in the mold halves are movable into alignment with each other so as to bring the dowel pins 32 into registration with the openings 33, and provided with suitable means for holding the halves 22 and 24 together. 70 The thin adherent refractory coating 50 is of more or less permanent nature and need be renewed only at relatively long intervals, for instance, not more than once a day when the molds are used for continuous production. It may be 75

noted that this coating 50, besides forming a heat insulating coating reducing the rate of heat transfer between the metal being poured and the metal of the mold halves 22 and 24, also serves as a means for preventing the molten metal from wearing away any sharp edges of the metal defining the mold depressions. The halves 22 and 24 having been clamped together, the various surfaces of the depressions are then coated with the lampblack previously referred to and molten metal is introduced into one end of the channel 36 where it flows down the trough 38 and successively fills the mold depressions. Preferably, only enough of such metal is introduced into the channel 36 as to fill only the depressions 34 and a portion of the depressions 35, thus effecting a saving in the amount of scrap resulting from the molding operation.

While the exact composition of the cast iron employed for forming the tappet is more or less unimportant in accordance with the broader aspects of the present invention as long as it is capable of producing a chilled or white cast iron face of the desired hardness for the tappet, I prefer to employ a cast iron having approximately the following composition:

|                 | Per cent      |
|-----------------|---------------|
| Silicon         | 2½            |
| Carbon          | 3½            |
| 30 Manganese    | .06           |
| Sulphur         | less than 1   |
| Phosphorus      | less than .25 |
| Remainder iron. |               |

35 It will be apparent when the molten cast iron is poured into the mold such iron will be insulated from direct contact with the surfaces of the depressions 34 by the heat insulating coating 50 but will come into direct contact with the upper surface of the chill plate 42 except for the relatively thin coating of lampblack previously referred to and which offers very little resistance to the transfer of heat through it. Accordingly, with the composition of iron referred to or an equivalent composition as far as the chilling characteristic thereof is concerned, that portion of the molten cast iron coming into contact with the chill plate 42 will be solidified so quickly as to prevent segregation of the carbon in the iron and the 40 face of the tappet will, accordingly, be formed from what is generally known as white cast iron which is of extreme hardness, while the body of the tappet is being insulated from the rapid absorption of heat therefrom, will permit a greater or lesser degree of segregation of the carbon in the metal and, accordingly, the body of the tappet will remain relatively soft. In actual operation castings are repeatedly made in the molds until the temperature of the halves 22 and 24 reaches a temperature of 400 degrees F. to 500 degrees F. or higher and until the temperature of the chill plate 42 reaches the neighborhood of about 300 degrees F. and thereafter the temperature of the chill plate 42 is maintained as near 45 to 350 degrees F. as possible and not to exceed 400 degrees F. If the temperature raises above this value, suitable means for cooling the chill plate and/or mold may be employed, as for instance cold air directed against the face of the mold and 50 chill plate until the temperature falls to the desired point. The chill plate 42 being greatly exposed upon separation of the halves 22 and 24, offers a relatively great area for contact with the cooling air upon separation of the halves and 55 consequently may be normally maintained at the

desired temperature by thus directing air against it when the halves are separated between casting operations. The mold halves themselves being of greater bulk than the chill plate, are not cooled to the same extent as the chill plate and consequently the temperature remains higher. Should, for any reason or another, the temperature of the chill plate 42 exceed the desired maximum temperature, it may be simply lifted out of place and replaced by another and cooler chill plate and 10 the operation continued uninterrupted. I have found that when the temperature of the chill plate 42 as determined by the thermo-couple 52 is maintained between 300 degrees and 400 degrees F. and preferably as closely as possible to 15 350 degrees F., the surface of the tappet when formed from the composition of iron given has a Brinell hardness reading between 300 and 400 or higher, corresponding to a Rockwell reading in excess of 37, which is a satisfactory degree of 20 hardness to insure a long life and little wear of the face of the tappet. Also that if the mean temperature of the mold halves 22 and 24 is kept above 400 degrees F. and up to 500 degrees F. or over, the main body portion of the tappet will be 25 sufficiently easily machinable to permit turning of its outer surface and drilling and tapping its end surface 16 for the reception of the usual adjusting screw (not shown).

It will, of course, be apparent that when the 30 molds are separated, the individual tappet castings are removed, the gates 20 are broken off or otherwise removed, the body and end portion 16 of the tappet is machined and the face of the head 12 ground where necessary to bring its surface into the desired final condition.

In the following claims the phrase "continued production—by repeatedly casting—in a mold" or equivalent phrase is to be interpreted to mean such continued use of a mold in casting operations that it does not have the opportunity to cool to room temperature between each pouring of metal thereinto.

It will, of course, be apparent that certain steps of operation herein described and disclosed may 45 be varied to a greater or lesser extent without departing from the spirit and substance of the broad invention, the scope of which is commensurate with the appended claims.

I claim:

1. In the continued production of cast iron members having a chilled face by repeatedly casting molten cast iron of a type adapted to form white cast iron when chilled into a metallic mold having a separate chill plate, the step of artificially cooling the chill plate to maintain its average temperature between 300° F. and 400° F. during the casting operations.

2. In the continued production of cast iron members having a chilled face by repeatedly casting molten cast iron of a type adapted to form white cast iron when chilled into a metallic mold having a separate chill plate, the step of maintaining the temperature of the chill plate between 300° F. and 400° F. and the temperature of the mold in excess of 400° F. during the casting operations.

3. In the continued production of cast iron members having a chilled face by repeatedly casting molten cast iron of a type adapted to form white cast iron when chilled into a metallic mold having a separate chill plate, the steps of heating the mold to above 400° F. and the chill plate to above 300° F., and then limiting the max- 75

imum temperature of the chill plate to approximately 400° F. during the casting operations.

4. In the continued production of cast iron valve tappets from molten cast iron of a type adapted to form white cast iron when chilled by the use of a metallic mold having a removable uninsulated chill plate, the steps of heating the chill plate to above 300° F. by repeated casting operations and replacing it with a cooler 10 chill plate when its temperature exceeds approximately 400° F.

5. In the continued production of cast iron valve tappets from molten cast iron of a type adapted to form white cast iron when chilled by the use of a metallic mold having a removable 15 uninsulated chill plate, the steps of heating the chill plate to above 300° F. by repeated casting operations and replacing it with a cooler chill

plate when its temperature exceeds approximately 400° F., and insulating the surfaces of the mold cavities other than the chill plate against the transfer of heat to the mold.

6. In the continued production of cast iron 5 articles having a relatively soft machinable portion and a chilled portion by repeatedly casting molten cast iron, of a type adapted to form white cast iron when chilled, in a metallic mold having a separate chill plate for said chilled portion, the steps of maintaining the temperature of the mold at a sufficiently high value to prevent chilling of the surfaces of the article formed thereby, and artificially cooling said chill plate to maintain the temperature thereof sufficiently 10 low to insure chilling of the surface of the article formed thereby.

JOSEPH L. DOSTAL.